

No. 697,408.

Patented Apr. 8, 1902.

E. HUBBARD.

SPOOL AND PROCESS OF PRODUCING SAME.

(Application filed Aug. 14, 1901.)

(No Model.)

Fig. 1.



Fig. 5



Fig. 2.



Fig. 3.



Fig. 4.



Fig. 6.



Witnesses.

Edward T. Wray.

Adna H. Bowen, Jr.

Inventor:  
E. Hubbard  
by Burton Burton  
Kiss Atty's.

# UNITED STATES PATENT OFFICE.

EBER HUBBARD, OF CHICAGO, ILLINOIS.

## SPOOL AND PROCESS OF PRODUCING SAME.

SPECIFICATION forming part of Letters Patent No. 697,408, dated April 8, 1902.

Application filed August 14, 1901. Serial No. 71,981. (No model.)

To all whom it may concern:

Be it known that I, EBER HUBBARD, a citizen of the United States, residing at Chicago, in the county of Cook and State of Illinois, have invented certain new and useful Improvements in Spools and Processes of Producing the Same, of which the following is a specification, reference being had to the accompanying drawings, forming a part thereof.

The purpose of this invention is to provide a spool which is made substantially of fibrous pulp, which can be produced cheaply and will have sufficient strength and hardness to endure the process of winding on it the thread which it is to carry as tightly as such thread should be wound, and having also sufficient stubbornness of texture, particularly at the center, to adapt it to be held firmly and securely and centered accurately by the device on which it is necessary that it should be mounted in order to receive the rotary motion necessary for winding the thread upon it.

All attempts at producing from fibrous pulp the large spools upon which the thread is wound for manufacturers' use have been unsuccessful, because of the difficulty experienced in preventing the molding of a spool from pulp of sufficient and sufficiently uniform density and tenacity to prevent it, on the one hand, from being crushed or distorted by the tension of the thread wound about it, and on the other hand being ruptured by the longitudinal strain and the torsional strain to which it is subjected in such winding.

The great difficulty in the way of molding a spool of fibrous pulp of sufficiently uniform density arises from the great difference in the radial depth of the pulp at the barrel and at the heads, respectively, of the spool, such difference tending to prevent the full drainage of the water from the pulp at the two parts, differing so greatly in thickness or depth of the two parts to be drained. The difficulty in the way of producing a satisfactory spool from fibrous pulp arises from its lack of tenacity longitudinally and the necessity for reinforcing it in some manner to increase such tenacity. This has usually been attempted by providing it with some sort of a core of other material than the molded pulp, and herein the difficulty experienced arises in securely combining such core with the

pulp, so as to produce a thoroughly-coherent structure and at the same time one which can be produced inexpensively.

55

I have overcome both the difficulties above indicated by the process of manufacturing a fibrous pulp spool of the form and structure hereinafter described.

In the drawings, Figure 1 is an axial section 60 of my improved spool. Fig. 2 is an end elevation of the spool-body of fibrous pulp without the reinforcing wooden core. Fig. 3 is a similar end elevation, showing one of the wooden strips which is to constitute the star-shaped core in the position in which it is ready to be forced "home" into the recess provided for it in the molded fiber-body. Fig. 4 is a similar end elevation showing all the five wooden strips which together constitute the 65 reinforcing wooden core in position ready to be forced home, but not yet forced into final position. Fig. 5 is an end elevation of the complete spool, showing the wooden strips forced home into the recesses provided for them in the molded body of the spool. Fig. 70 75

6 is a perspective view representing the manner of forcing the strips which constitute the wooden core radially outward into full seating and final position in the recesses formed 80

for them in the molded pulp-body, and showing the mandrel used for that purpose introduced and ready to be forced through the axial aperture of the spool to crowd the strips 85

into position. 85

A represents the fibrous pulp-body of the spool, which is molded with a star-shaped axial aperture A'. (See Fig. 2.) This star-shaped aperture affords, as will be seen, a very large area for drainage of the water out of the pulp 90 as it is compressed in the mold provided for that purpose, with the result that the central portion of the spool when the molding of the same is complete is as thoroughly hard and compact and tenacious as the outer surface. 95 This result could not be obtained if the spool were made merely with a cylindrical aperture, for, as is well understood by those accustomed to operating with fibrous pulp in molds, the fiber will be laid most compactly 100 at the surfaces to which the freest drainage of water is provided, and wherever there is insufficient surface for drainage there the pulp will remain moist and will become spongy

when the article is dried to hardness. When the spool - body of fibrous pulp has been molded in the form indicated in Fig. 2, it is dried to hardness, and the star-shaped cavity 5 is first filled with glue, and the glue is then allowed to drain from it, leaving all the surfaces of said cavity coated with glue. If the wooden reinforce or core which is to occupy the star-shaped cavity and completely fill it, 10 making junction with all its surfaces, were now introduced endwise into such cavity, the glue would be completely scraped from the surfaces and no adequate junction or union by adhesion would occur between the pulp-body 15 and the wooden core. I avoid thus scraping the glue from the surface to which adhesion is desired by making the wooden core, consisting of separate strips, each adapted to enter one of the wedge-shaped recesses  $a'$   $a'$  of the star-shaped total recess  $A'$ , and each of these wedge-shaped strips  $B$  is adapted to be entered longitudinally through the open center of the spool without necessarily touching the surface of the star-shaped cavity at any point; but 20 having thus been introduced longitudinally it may be moved out radially edgewise into one of the wedge-shaped recesses  $a'$ , and in such movement its lateral surfaces, which are to be joined by the glue to the surfaces of the 25 recess, advance into contact with the latter surfaces without any tendency to scrape the glue therefrom. Each of the wedge-shaped strips  $B$   $B$   $B$   $B$   $B$  is in turn introduced into the star-shaped cavity and passed out edgewise into one of the recesses until all are assembled in the manner appearing in Fig. 4, 30 in which it will be noticed that the strips  $B$   $B$   $B$ , &c., are not yet forced out into perfect contact with the surfaces of the recesses  $a'$ . When they are all thus assembled, a cylindrical mandrel  $C$ , having, preferably, a slightly-tapered end, is introduced within the 35 group of strips  $B$   $B$   $B$  and forced longitudinally through the whole length of the spool, its diameter being such that as it passes 40 through the center of the spool it forces all the strips out edgewise and crowds them tightly into the recesses, respectively, into 45

which they are lodged, forcing out any excess of glue at the end and insuring a perfect union between the strips and the pulp-body. 50

I claim—

1. The process of making a spool of fibrous pulp which consists of the following steps, to wit: first, molding a pulp-body with an axial aperture having recesses leading radially from it along its entire length, wedge-shaped in transverse section of the spool; second, drying such pulp-body to hardness; third, applying glue to the inner surfaces of such wedge-shaped radial recesses; fourth, introducing endwise through the axial aperture and entering edgewise into the recesses respectively wood strips or bars wedge-shaped in cross-section; fifth, passing longitudinally through 65 the axial aperture a cylindrical mandrel adapted to crowd all the wedge-shaped strips edgewise simultaneously into their respective apertures.

2. A spool, comprising a body molded of 70 fibrous pulp, with an axial aperture having recesses leading off radially from it along its entire length, and wooden strips glued in such recesses.

3. A spool of fibrous pulp, having through 75 its entire length a star-shaped wooden core with an axial aperture.

4. A spool, having a star-shaped wooden core with an axial aperture, and a pulp-body in which such core is embedded, such core 80 being composed of strips wedge-shaped in cross-section, arranged with their bases or wider edges encompassing the central aperture.

5. A spool-body of molded fibrous pulp, 85 having an axial star-shaped aperture extending from end to end.

In testimony whereof I have hereunto set my hand at Chicago, Illinois, in the presence of two witnesses, this 9th day of August, A. 90 D. 1901.

EBER HUBBARD.

In presence of—

ADNA H. BOWEN, Jr.,  
EDWARD T. WRAY.